

# UNITED STATES PATENT OFFICE.

JOHN DRAPER, OF BROOKLYN, NEW YORK.

## PROCESS OF REMOVING SCALES FROM BOILERS.

SPECIFICATION forming part of Letters Patent No. 509,209, dated November 21, 1893.

Application filed March 1, 1892. Serial No. 423,404. (No specimens.) Patented in England May 12, 1891, No. 8,115, and January 12, 1892, No. 607.

*To all whom it may concern:*

Be it known that I, JOHN DRAPER, chemist, a citizen of the United States, residing at Thir-  
5 ty-eighth street, above Fifth avenue, Brook-  
lyn, New York, but at present residing at 4  
Albany Street, Kelvinside, Glasgow, in the  
county of Lanark, Scotland, have invented cer-  
tain new and useful improvements in methods  
of and means for removing and preventing  
10 scales or incrustations in steam-boilers, and  
for the prevention of pitting, corrosion, or  
oxidation of such boilers, which improvements  
are also applicable to the coating of iron or  
steel articles generally so as to protect them  
15 from oxidation, (for which I have received  
Letters Patent in England, No. 8,115, dated  
May 12, 1891, and No. 607, dated January 12,  
1892;) and I do hereby declare that the follow-  
20 ing is a full, clear, and exact description of the  
invention, which will enable others skilled in  
the art to which it appertains to make and use  
the same.

This invention relates to means for removing  
25 scales or incrustations from steam boil-  
ers, and for the prevention of pitting, corro-  
sion, or oxidation of such boilers, the invention  
being also applicable to the coating of iron or  
steel articles generally so as to protect them  
30 from oxidation, and it consists broadly  
in coating the surface which it is desired to  
protect with a thin film of oxide of mercury.

According to the method of carrying out  
my invention I employ metallic mercury and  
metallic sodium or potassium, and carbonate  
35 of sodium or potassium, which when placed  
in a closed vessel of iron or steel containing  
water, will under the action of heat and pres-  
sure deposit a thin film or coating upon the  
walls of such vessel, and thereby protect same  
40 from pitting, corrosion and oxidation, and  
will also prevent the formation of scales or  
incrustations thereon, while in the case of  
boilers or other vessels upon the walls of which  
scales or incrustations are already formed,  
45 the use of such materials will in a compara-  
tively short time effectually remove the same.  
Further, by placing or suspending iron or steel  
articles generally, in the boiler or vessel con-  
taining water into which the materials above  
50 mentioned have been introduced, when the  
boiler or vessel is heated such articles will

within a comparatively short period become  
coated with a thin film of such a nature as to  
effectually resist oxidation, and so protect  
such articles. The quantities of the mate-  
55 rials above named which it is necessary to  
use are immaterial, some excess doing no in-  
jury, and the proportions may vary within  
large limits and will depend upon the nature  
of the water employed and other circum-  
60 stances, but I find that ten ounces of mercury  
to one ounce of sodium, with sufficient carbon-  
ate of sodium or of potassium to produce by  
itself alkaline reaction in the water contained  
in the boiler or vessel, and which being in the  
65 form of a carbonate will produce better re-  
sults than the alkali produced by the decom-  
position of the sodium present will in most  
cases be ample for every five hundred square  
feet of surface to be coated.

The mercury is first mixed with the sodium  
metal and a hard amalgam is formed if mixed  
in the proportions stated. This amalgam is  
introduced into the water of the boiler, and  
by the time the boiler is under steam the de-  
70 composition of the sodium has liberated the  
mercury slowly and in extremely fine parti-  
cles, which division of the mercury is neces-  
sary to secure the oxidation to form the coat-  
ing. The sodium, apart from its value in hold-  
75 ing the mercury and liberating it in fine par-  
ticles, is of great value on account of the ease  
with which it forms caustic soda with the wa-  
ter of the boiler, thereby greatly assisting in  
the oxidation of the mercury under pressure  
80 and heat, as well as its effect upon the boiler-  
plates, cleansing them from grease and other  
objectionable substances. The carbonate of  
soda is found necessary to supply sufficient  
alkali to the water, first on account of the  
85 great difficulty found in depositing upon the  
surface of iron or steel a coating of oxide of  
mercury unless the water be slightly alka-  
line, and secondly it has a specific effect in  
neutralizing any acidity frequently found in  
90 some boiler waters. The process in practice  
is therefore:—The introduction of an amal-  
gam of mercury and sodium in the stated  
proportions into a boiler, the raising of the  
water contained in the boiler to the working  
95 pressure (which may be fifty to eighty pounds  
per square inch), the introduction into the

water of the boiler by the feed of sufficient carbonate to cause the water to be alkaline. If the water is kept in this condition the gradual liberation of the mercury is brought about 5 by the decomposition of the mercury-sodium amalgam and is oxidized to an oxide of mercury in contact with a carbonate and with the assistance of the caustic soda. The process being carried out as described and the 10 boiler kept in working condition, the time required to produce the best effect, while it differs in nearly every case according to the conditions, will be approximately not more than six months nor less than three months. 15 The patent of the United States No. 453,882 issued to myself and Alfred Holmgren, Henry Mount and John Barnes, describes the use of water, bichloride of mercury, mercury and sodium, under heat and pressure for the purpose 20 of coating the internal surfaces of steam boilers to prevent incrustation. It has been found almost impossible to apply the coating or enamel to the boiler plate from that composition in boilers which have a tendency 25 from various causes such as acid feed waters, &c., to rusting, corrosion or wasting away of the plate. In order to successfully apply the coating it is necessary that the water be kept slightly alkaline and sufficient alkali is not 30 produced in the process described by the previous patent cited, by the decomposition of metallic sodium to maintain the required alkalinity. It would be commercially impracticable to use sufficient metallic sodium to 35 bring about the necessary state of alkalinity

on account of the cost thereof. Moreover, in the working of the former patent it was necessary to put in the materials in two operations, to wit: (first) to dissolve the  $HgCl_2$  in the water of the boiler, and (second) to add 40 the mercury and sodium to the solution thus formed. In the present case a free alkali is used, all the materials are compounded together, and the whole operation is performed at once. 45

Referring again to boilers liable to corrosion, the amount of free alkali necessary makes it impossible to use the mercury bichloride of the former patent on account of the decomposition expressed in the reaction 50 as follows:



Having fully described my invention, what I claim, and desire to secure by Letters Patent, is—

The method of treating iron or steel surfaces so as to protect them from pitting, corrosion, or oxidation, or prevent the formation of scales or incrustations thereon, or to remove the same therefrom, consisting in subjecting such surfaces to the action of water, metallic mercury and metallic sodium or potassium and carbonate of sodium or of potassium under heat and pressure, as set forth. 65

JOHN DRAPER.

Witnesses:

CHAS. A. ALLISON,  
HARRY A. MCLELLAN.